

July 22, 1947.

J. E. WHITE

2,424,294

GRAPHITE OUTGASSING

Filed March 1, 1945

Fig. 1.



Fig. 2.

TO VACUUM SYSTEM



INVENTOR  
J. E. WHITE

BY *J. E. White*  
ATTORNEY

## UNITED STATES PATENT OFFICE

2,424,294

## GRAPHITE OUTGASSING

John E. White, Bloomfield, N. J., assignor to  
Westinghouse Electric Corporation, East Pitts-  
burgh, Pa., a corporation of Pennsylvania

Application March 1, 1945, Serial No. 580,357

4 Claims. (Cl. 316—21)

1

This invention relates to graphite outgassing and has particular application to the electronic art and outgassing of such graphite parts as anodes, baffles and the like, which are used within an evacuated electronic device.

It is well appreciated in the electronic art that graphite parts have a tendency to release gas therefrom into an evacuated container in which situated particularly when said part becomes heated in use. Presence of gas in an electronic device will not only change its characteristics but in most instances renders the device inoperative for its intended purposes. For instance, an ignitron utilizes a graphite anode, and in use may be subjected to intense heat at some spot from an arc back. If the heat at that spot liberates gas from the anode, the gas will result in greater ionization in the ignitron, which in turn encourages further arc backs with the probability of release of further gas from the anode. Thus the ignitron becomes progressively worse and soon is useless for its intended purpose.

Broadly considered, therefore, the invention has for an object the more perfect outgassing of graphite parts.

Likewise, from its most general aspect, the invention proposes the outgassing of graphite parts at temperatures exceeding any encountered in use.

A further object of the invention is to protect the graphite part after it is outgassed and until incorporated in the electronic device so it may be then finally and adequately outgassed by normal procedure with other parts of the device.

Still further objects of the invention will appear to those skilled in the art to which it appertains as the description progresses, both by direct recitation thereof and by implication from the context.

In the accompanying drawing:

Figure 1 illustrates an ignitron having an anode of the character treated in accordance with the present invention; and

Figure 2 is a sectional view of an apparatus for carrying out the outgassing of graphite parts in accordance with the invention.

By way of example, an ignitron is shown in Figure 1 having a graphite anode 10 suspended in a sealed envelope 11 on the bottom header 12 of which is a mercury pool cathode 13 into which a starter electrode or ignitor 14 is dipped. During manufacture of the ignitron, the same is subjected to as high a temperature as the character of its parts and joints will permit, for purposes of freeing gas from internal parts and while the de-

2

vice is on the pumps being evacuated. Since the ignitron must of necessity contain parts having lower melting temperatures than those of the anode or its envelope, there is a practical limitation on heat which can be safely applied to the anode after it is mounted in the ignitron. Unfortunately, the limitation is too low to permit heating the anode to sufficiently high temperature to thoroughly outgas it. Attempts have been heretofore made to outgas the anode before introducing it into the ignitron, but it has been found that the outgassed anode when exposed to air in making transfer to the ignitron, absorbs gasses from the air, which again so contaminate the anode that normal outgassing in the ignitron envelope does not suffice.

According to the present invention, the graphite part, and in the present instance, the anode 10 as representative of such part, is treated prior to being applied in intended place of use within the envelope. An electric furnace 15 is shown in Figure 2 for the purpose, said furnace having a temporarily sealed shell 16 which is surrounded by a cooling coil 17 that the exterior may not become injuriously hot to the detriment of the furnace. Within the shell is a heating element 18 of hollow formation to constitute the oven, and between the heating element or oven and the several walls of the shell are heat shields 19 serving to confine the greater part of the developed heat to the oven. The part, such as anode 10, to be outgassed is placed in the oven. Lead-in connections 20 pass current to the heating element or oven and by it a temperature within the range of 1800° C. to 2000° C. is developed in the oven and effective upon part 10.

Shell 16 has a pipe connection 21 to its interior from the exterior, and during the heating period above related, this pipe connection is joined, as 40 through a valve 22 to a vacuum pump or system by which the oven is evacuated. The part 10 can be considered degassed when the pressure goes down to .75 micron at 1800° C. and when the pumps can be shut off for one hour at 1800° C. without the pressure rising above 3 microns.

When the degassing has thus been accomplished, the temperature in the oven is reduced to 200° C. or less, to be within a temperature range wherein an appropriate gas to be used, 50 such as hydrogen, or one of the noble gases such as helium, argon, neon, and so forth, is practically insoluble in solids. For brevity, the selected gas will be referred to as the protective gas. At that temperature condition of the oven, the valve 22 55 (which for the purpose is preferably a three-

way valve) is turned to admit the said protective gas to the oven and fill the same to atmospheric pressure. The protective gas at this temperature and pressure enters the surface pores of the part 10 outgassed. The protective gas does not seem to penetrate to any considerable depth, and yet by surface absorption or impregnation thereof in the anode, it constitutes a protection against extraneous gases being absorbed when the anode is next exposed to air. This surface penetration of the protective gas is readily removed by subsequent normal outgassing procedure applied to the ignitron after transfer of the anode to its appointed place therein. As indicated above, hydrogen and the noble gases are not dissolved in graphite to any objectionable extent, and those gases are therefore readily removed at moderate temperatures. Such small amount of hydrogen as may have dissolved in the graphite, on being released during the higher temperature periods during exhaust, has a beneficial effect in removing traces of injurious oxides which may have been left in the tube inadvertently.

Consequently, after the hydrogen or other protective gas has been introduced into the oven as above recited, the protective gas supply is shut off and the furnace shell opened. The graphite part or anode 10 is then promptly transferred to its appointed place, as in the ignitron envelope, and that envelope, with its contents, then subjected to the usual outgassing procedure. In this stage of operation, temperatures from about 800° C. and not exceeding 1200° C. are usually employed while the device is on the pump for evacuating said device or ignition in the present instance. The protective surface infiltration of hydrogen or other protective gas present in the graphite part due to the pre-mounting and outgassing procedure outlined above, is readily drawn from the anode at this lower temperature approximating 800° C. to 1200° C., and thus the anode is to all intents and purposes devoid of releasable gas. As a result, arc-back spots in use on the anode, which are at a lower temperature than the primary outgassing temperature of 1800° C. to 2000° C., have no gas-releasing effect, and the ignitron remains in good evacuated condition free of evolved gas from the arc back.

While the foregoing description has utilized graphite as an exemplary material being outgassed and has referred to the part as an anode and as used in an ignitron as the device in which used, the invention is to be understood as also applicable to other materials, parts and devices.

I claim:

1. An outgassing method for a part to be used in an evacuated envelope, comprising outgassing the part at a temperature approximating 1800° C., applying a surface impregnation of a protective gas to the outgassed part, enclosing said part in an envelope, and outgassing said part in said envelope at a less temperature than before.
2. An outgassing method for a part to be used in an evacuated envelope, comprising outgassing the part at a temperature in the approximate range of 1800° C. to 2000° C., reducing the temperature to approximately a tenth of the said outgassing temperature, applying a protective gas to the part at its reduced temperature, enclosing said part in an envelope and outgassing said part in said envelope at a less temperature than the first used outgassing temperature.
3. An outgassing method for a part to be used in an evacuated envelope, comprising outgassing the part before introduction into said envelope at a temperature in the approximate range of 1800° C. to 2000° C., reducing the temperature to approximately 200° C., applying hydrogen as a protective surface impregnation to said part at its reduced temperature, transferring said part to and mounting it in an envelope for use, and again outgassing said part and in its final position in said envelope and at a temperature less than the said range of 1800° C. to 2000° C. and more than the approximate said temperature of 200° C. at which the hydrogen was applied.
4. An outgassing method for a part to be used in an evacuated envelope, comprising heating the part in vacuum to a temperature less than its melting point and simultaneously outgassing the same before introduction into said envelope, cooling said part while still in vacuum, and after cooling of said part admitting a protecting gas thereto, transferring said part to said envelope, and again heating, but at a lower temperature than the first said heating, and simultaneously outgassing said part in the envelope.

JOHN E. WHITE.

#### REFERENCES CITED

The following references are of record in the file of this patent:

#### UNITED STATES PATENTS

| Number    | Name    | Date          |
|-----------|---------|---------------|
| 2,184,323 | Spanner | Dec. 26, 1939 |